



US005540150A

**United States Patent** [19]

Lewis et al.

[11] **Patent Number:** 5,540,150[45] **Date of Patent:** \* Jul. 30, 1996[54] **LASER-DRIVEN METHOD AND APPARATUS FOR LITHOGRAPHIC IMAGING AND PRINTING PLATES FOR USE THEREWITH**

[75] Inventors: **Thomas E. Lewis**, E. Hampstead; **Richard A. Williams**, Hampstead; **Frank G. Pensavecchia**, Hudson; **John F. Kline**; **John P. Gardiner**, both of Londonderry, all of N.H.; **Michael T. Nowak**, Leominster; **Kenneth T. Robichaud**, Fitchburg, both of Mass.

[73] Assignee: **Presstek, Inc.**, Hudson, N.H.

[\*] Notice: The portion of the term of this patent subsequent to Jan. 31, 2012, has been disclaimed.

[21] Appl. No.: 380,805

[22] Filed: Jan. 30, 1995

**Related U.S. Application Data**

[63] Continuation of Ser. No. 159,955, Nov. 29, 1993, Pat. No. 5,385,092, which is a continuation of Ser. No. 917,481, Jul. 20, 1992, abandoned.

[51] **Int. Cl.<sup>6</sup>** ..... B41N 1/14; B41C 1/10; B41M 5/24

[52] **U.S. Cl.** ..... 101/467; 101/453; 101/457; 101/462; 430/303; 430/326

[58] **Field of Search** ..... 101/453, 454, 101/456, 457, 458, 459, 460, 461, 462, 463.1, 465-467, 395, 401.1; 430/303, 325, 326, 329

[56]

**References Cited****U.S. PATENT DOCUMENTS**

|           |         |                          |           |
|-----------|---------|--------------------------|-----------|
| 3,677,178 | 7/1972  | Gipe .....               | 101/450.1 |
| 4,063,949 | 12/1977 | Uhlig et al. ....        | 101/467   |
| 4,347,785 | 9/1982  | Chase et al. ....        | 101/467   |
| 4,395,946 | 8/1983  | Price .....              | 101/457   |
| 4,842,988 | 6/1989  | Herrmann et al. ....     | 430/14    |
| 4,842,990 | 6/1989  | Herrmann et al. ....     | 430/272   |
| 4,861,698 | 8/1989  | Hiruma et al. ....       | 101/467   |
| 4,936,211 | 6/1990  | Pensavecchia et al. .... | 101/136   |
| 5,053,311 | 10/1991 | Makino et al. ....       | 430/166   |
| 5,148,746 | 9/1992  | Fuller et al. ....       | 101/142   |
| 5,259,311 | 11/1993 | McCaughay, Jr. ....      | 101/401.1 |

**FOREIGN PATENT DOCUMENTS**

1050805 3/1974 Canada .

**OTHER PUBLICATIONS**

Nechiporenko et al., "Direct Method of Producing Waterless Offset Plates By Controlled Laser Beam". Research Disclosure, Apr. 1980, at p. 131.

*Primary Examiner*—Stephen Funk  
*Attorney, Agent, or Firm*—Cesari and McKenna

[57] **ABSTRACT**

Apparatus and methods for imaging lithographic plates using laser devices that emit in the near-infrared region, and plates suitable for imaging with the apparatus and methods. Laser output either ablates one or more plate layers or physically transforms a surface layer, in either case resulting in an imagewise pattern of features on the plate. The image features exhibit an affinity for ink or an ink-abhesive fluid that differs from that of unexposed areas.

44 Claims, 5 Drawing Sheets







FIG.10



FIG.4



FIG.5

FIG.6





FIG. 7



FIG. 8



FIG. 9



FIG. 11



FIG. 12



FIG. 13



FIG. 14



FIG. 15



FIG. 16

**LASER-DRIVEN METHOD AND APPARATUS  
FOR LITHOGRAPHIC IMAGING AND  
PRINTING PLATES FOR USE THEREWITH**

**RELATED APPLICATION**

This is a continuation of Ser. No. 08/159,955, filed Nov. 29, 1993, now U.S. Pat. No. 5,385,092, which is itself a continuation of Ser. No. 07/917,481, filed Jul. 20, 1992, now abandoned.

**BACKGROUND OF THE INVENTION**

**A. Field of the Invention**

The present invention relates to digital printing apparatus and methods, and more particularly to a system for imaging lithographic printing plates on- or off-press using digitally controlled laser output.

**B. Description of the Related Art**

Traditional techniques of introducing a printed image onto a recording material include letterpress printing, gravure printing and offset lithography. All of these printing methods require a plate, usually loaded onto a plate cylinder of a rotary press for efficiency, to transfer ink in the pattern of the image. In letterpress printing, the image pattern is represented on the plate in the form of raised areas that accept ink and transfer it onto the recording medium by impression. Gravure printing cylinders, in contrast, contain series of wells or indentations that accept ink for deposit onto the recording medium; excess ink must be removed from the cylinder by a doctor blade or similar device prior to contact between the cylinder and the recording medium.

In the case of offset lithography, the image is present on a plate or mat as a pattern of ink-accepting (oleophilic) and ink-repellent (oleophobic) surface areas. In a dry printing system, the plate is simply inked and the image transferred onto a recording material; the plate first makes contact with a compliant intermediate surface called a blanket cylinder which, in turn, applies the image to the paper or other recording medium. In typical sheet-fed press systems, the recording medium is pinned to an impression cylinder, which brings it into contact with the blanket cylinder.

In a wet lithographic system, the non-image areas are hydrophilic, and the necessary ink-repellency is provided by an initial application of a dampening (or "fountain") solution to the plate prior to inking. The ink-abhesive fountain solution prevents ink from adhering to the non-image areas, but does not affect the oleophilic character of the image areas.

If a press is to print in more than one color, a separate printing plate corresponding to each color is required, each such plate usually being made photographically as described below. In addition to preparing the appropriate plates for the different colors, the operator must mount the plates properly on the plate cylinders of the press, and coordinate the positions of the cylinders so that the color components printed by the different cylinders will be in register on the printed copies. Each set of cylinders associated with a particular color on a press is usually referred to as a printing station.

In most conventional presses, the printing stations are arranged in a straight or "in-line" configuration. Each such station typically includes an impression cylinder, a blanket cylinder, a plate cylinder and the necessary ink (and, in wet systems, dampening) assemblies. The recording material is transferred among the print stations sequentially, each sta-

tion applying a different ink color to the material to produce a composite multi-color image. Another configuration, described in U.S. Pat. No. 4,936,211 (co-owned with the present application and hereby incorporated by reference), relies on a central impression cylinder that carries a sheet of recording material past each print station, eliminating the need for mechanical transfer of the medium to each print station.

With either type of press, the recording medium can be supplied to the print stations in the form of cut sheets or a continuous "web" of material. The number of print stations on a press depends on the type of document to be printed. For mass copying of text or simple monochrome line-art, a single print station may suffice. To achieve full tonal rendition of more complex monochrome images, it is customary to employ a "duotone" approach, in which two stations apply different densities of the same color or shade. Full-color presses apply ink according to a selected color model, the most common being based on cyan, magenta, yellow and black (the "CMYK" model). Accordingly, the CMYK model requires a minimum of four print stations; more may be required if a particular color is to be emphasized. The press may contain another station to apply spot lacquer to various portions of the printed document, and may also feature one or more "perfecting" assemblies that invert the recording medium to obtain two-sided printing.

The plates for an offset press are usually produced photographically. To prepare a wet plate using a typical negative-working subtractive process, the original document is photographed to produce a photographic negative. This negative is placed on an aluminum plate having a water-receptive oxide surface coated with a photopolymer. Upon exposure to light or other radiation through the negative, the areas of the coating that received radiation (corresponding to the dark or printed areas of the original) cure to a durable oleophilic state. The plate is then subjected to a developing process that removes the uncured areas of the coating (i.e., those which did not receive radiation, corresponding to the non-image or background areas of the original), exposing the hydrophilic surface of the aluminum plate.

A similar photographic process is used to create dry plates, which typically include an ink-abhesive (e.g., silicone) surface layer coated onto a photosensitive layer, which is itself coated onto a substrate of suitable stability (e.g., an aluminum sheet). Upon exposure to actinic radiation, the photosensitive layer cures to a state that destroys its bonding to the surface layer. After exposure, a treatment is applied to deactivate the photoresponse of the photosensitive layer in unexposed areas and to further improve anchorage of the surface layer to these areas. Immersion of the exposed plate in developer results in dissolution and removal of the surface layer at those portions of the plate surface that have received radiation, thereby exposing the ink-receptive, cured photosensitive layer.

Photographic platemaking processes tend to be time-consuming and require facilities and equipment adequate to support the necessary chemistry. To circumvent these shortcomings, practitioners have developed a number of electronic alternatives to plate imaging, some of which can be utilized on-press. With these systems, digitally controlled devices alter the ink-receptivity of blank plates in a pattern representative of the image to be printed. Such imaging devices include sources of electromagnetic-radiation pulses, produced by one or more laser or non-laser sources, that create chemical changes on plate blanks (thereby eliminating the need for a photographic negative); ink-jet equipment that directly deposits ink-repellent or ink-accepting spots on

plate blanks; and spark-discharge equipment, in which an electrode in contact with or spaced close to a plate blank produces electrical sparks to physically alter the topology of the plate blank, thereby producing "dots" which collectively form a desired image (see, e.g., U.S. Pat. No. 4,911,075, co-owned with the present application and hereby incorporated by reference).

Because of the ready availability of laser equipment and their amenability to digital control, significant effort has been devoted to the development of laser-based imaging systems. Early examples utilized lasers to etch away material from a plate blank to form an intaglio or letterpress pattern. See, e.g., U.S. Pat. Nos. 3,506,779; 4,347,785. This approach was later extended to production of lithographic plates, e.g., by removal of a hydrophilic surface to reveal an oleophilic underlayer. See, e.g., U.S. Pat. No. 4,054,094. These systems generally require high-power lasers, which are expensive and slow.

A second approach to laser imaging involves the use of thermal-transfer materials. See, e.g., U.S. Pat. Nos. 3,945,318; 3,962,513; 3,964,389; and 4,395,946. With these systems, a polymer sheet transparent to the radiation emitted by the laser is coated with a transferable material. During operation the transfer side of this construction is brought into contact with an acceptor sheet, and the transfer material is selectively irradiated through the transparent layer. Irradiation causes the transfer material to adhere preferentially to the acceptor sheet. The transfer and acceptor materials exhibit different affinities for fountain solution and/or ink, so that removal of the transparent layer together with unirradiated transfer material leaves a suitably imaged, finished plate. Typically, the transfer material is oleophilic and the acceptor material hydrophilic. Plates produced with transfer-type systems tend to exhibit short useful lifetimes due to the limited amount of material that can effectively be transferred. In addition, because the transfer process involves melting and resolidification of material, image quality tends to be visibly poorer than that obtainable with other methods.

Finally, lasers can be used to expose a photosensitive blank for traditional chemical processing. See, e.g., U.S. Pat. Nos. 3,506,779; 4,020,762. In an alternative to this approach, a laser has been employed to selectively remove, in an imagewise pattern, an opaque coating that overlies a photosensitive plate blank. The plate is then exposed to a source of radiation, with the unremoved material acting as a mask that prevents radiation from reaching underlying portions of the plate. See, e.g., U.S. Pat. No. 4,132,168. Either of these imaging techniques requires the cumbersome chemical processing associated with traditional, non-digital platemaking.

## DESCRIPTION OF THE INVENTION

### Brief Summary of the Invention

The present invention enables rapid, efficient production of lithographic printing plates using relatively inexpensive laser equipment that operates at low to moderate power levels. The imaging techniques described herein can be used in conjunction with a variety of plate-blank constructions, enabling production of "wet" plates that utilize fountain solution during printing or "dry" plates to which ink is applied directly.

A key aspect of the present invention lies in use of materials that enhance the ablative efficiency of the laser beam. Substances that do not heat rapidly or absorb significant amounts of radiation will not ablate unless they are

irradiated for relatively long intervals and/or receive high-power pulses; such physical limitations are commonly associated with lithographic-plate materials, and account for the prevalence of high-power lasers in the prior art.

In one embodiment of our invention, a suitable plate construction includes a first layer and a substrate underlying the first layer, the substrate being characterized by efficient absorption of infrared ("IR") radiation, and the first layer and substrate having different affinities for ink (in a dry-plate construction) or an adhesive fluid for ink (in a wet-plate construction). Laser radiation is absorbed by the substrate, and ablates the substrate surface/in contact with the first layer; this action disrupts the anchorage of the substrate to the overlying first layer, which is then easily removed at the points of exposure. The result of removal is an image spot whose affinity for the ink or ink-adhesive fluid differs from that of the unexposed first layer.

In a variation of this embodiment, the first layer, rather than the substrate, absorbs IR radiation. In this case the substrate serves a support function and provides contrasting affinity characteristics.

In both of these two-ply plate types, a single layer serves two separate functions, namely, absorption of IR radiation and interaction with ink or ink-adhesive fluid. In a second embodiment, these functions are performed by two separate layers. The first, topmost layer is chosen for its affinity for (or repulsion of) ink organ ink-adhesive fluid. Underlying the first layer is a second layer, which absorbs IR radiation. A strong, stable substrate underlies the second layer, and is characterized by an affinity for (or repulsion of) ink or an ink-adhesive fluid opposite to that of the first layer. Exposure of the plate to a laser pulse ablates the absorbing second layer, weakening the topmost layer as well. As a result of ablation of the second layer, the weakened surface layer is no longer anchored to an underlying layer, and is easily removed. The disrupted topmost layer (and any debris remaining from destruction of the absorptive second layer) is removed in a post-imaging cleaning step. This, once again, creates an image spot having a different affinity for the ink or ink-adhesive fluid than the unexposed first layer.

Post-imaging cleaning can be accomplished using a contact cleaning device such as a rotating brush (or other suitable means as described in U.S. Pat. No. 5,148,746, commonly owned with the present application and hereby incorporated by reference). Although post-imaging cleaning represents an additional processing step, the persistence of the topmost layer during imaging can actually prove beneficial. Ablation of the absorbing layer creates debris that can interfere with transmission of the laser beam (e.g., by depositing on a focusing lens or as an aerosol (or mist) of fine particles that partially blocks transmission). The disrupted but unremoved topmost layer prevents escape of this debris.

Either of the foregoing embodiments can be modified for more efficient performance by addition, beneath the absorbing layer, of an additional layer that reflects IR radiation. This additional layer reflects any radiation that penetrates the absorbing layer back through that-layer, so that the effective flux through the absorbing layer is significantly increased. The increase in effective flux improves imaging performance, reducing the power (that is, energy of the laser beam multiplied by its exposure time) necessary to ablate the absorbing layer. Of course, the reflective layer must either be removed along with the absorbing layer by action of the laser pulse, or instead serve as a printing surface instead of the substrate.

The imaging apparatus of the present invention includes at least one laser device that emits in the IR, and preferably near-IR region; as used herein, "near-IR" means imaging radiation whose  $\lambda_{max}$  lies between 700 and 1500 nm. An important feature of the present invention is the use of solid-state lasers (commonly termed semiconductor lasers and typically based on gallium aluminum arsenide compounds) as sources; these are distinctly economical and convenient, and may be used in conjunction with a variety of imaging devices. The use of near-IR radiation facilitates use of a wide range of organic and inorganic absorption compounds and, in particular, semiconductive and conductive types.

Laser output can be provided directly to the plate surface via lenses or other beam-guiding components, or transmitted to the surface of a blank printing plate from a remotely sited laser using a fiber-optic cable. A controller and associated positioning hardware maintains the beam output at a precise orientation with respect to the plate surface, scans the output over the surface, and activates the laser at positions adjacent selected points or areas of the plate. The controller responds to incoming image signals corresponding to the original document or picture being copied onto the plate to produce a precise negative or positive image of that original. The image signals are stored as a bitmap data file on a computer. Such files may be generated by a raster image processor (RIP) or other suitable means. For example, a RIP can accept input data in page-description language, which defines all of the features required to be transferred onto the printing plate, or as a combination of page-description language and one or more image data files. The bitmaps are constructed to define the hue of the color as well as screen frequencies and angles.

The imaging apparatus can operate on its own, functioning solely as a platemaker, or can be incorporated directly into a lithographic printing press. In the latter case, printing may commence immediately after application of the image to a blank plate, thereby reducing press set-up time considerably. The imaging apparatus can be configured as a flatbed recorder or as a drum recorder, with the lithographic plate blank mounted to the interior or exterior cylindrical surface of the drum. Obviously, the exterior drum design is more appropriate to use in situ, on a lithographic press, in which case the print cylinder itself constitutes the drum component of the recorder or plotter.

In the drum configuration, the requisite relative motion between the laser beam and the plate is achieved by rotating the drum (and the plate mounted thereon) about its axis and moving the beam parallel to the rotation axis, thereby scanning the plate circumferentially so the image "grows" in the axial direction. Alternatively, the beam can move parallel to the drum axis and, after each pass across the plate, increment angularly so that the image on the plate "grows" circumferentially. In both cases, after a complete scan by the beam, an image corresponding (positively or negatively) to the original document or picture will have been applied to the surface of the plate.

In the flatbed configuration, the beam is drawn across either axis of the plate, and is indexed along the other axis after each pass. Of course, the requisite relative motion between the beam and the plate may be produced by movement of the plate rather than (or in addition to) movement of the beam.

Regardless of the manner in which the beam is scanned, it is generally preferable (for reasons of speed) to employ a plurality of lasers and guide their outputs to a single writing array. The writing array is then indexed, after completion of

each pass across or along the plate, a distance determined by the number of beams emanating from the array, and by the desired resolution (i.e., the number of image points per unit length).

#### BRIEF DESCRIPTION OF THE DRAWINGS

The foregoing discussion will be understood more readily from the following detailed description of the invention, when taken in conjunction with the accompanying drawings, in which:

FIG. 1 is an isometric view of the cylindrical embodiment of an imaging apparatus in accordance with the present invention, and which operates in conjunction with a diagonal-array writing array;

FIG. 2 is a schematic depiction of the embodiment shown in FIG. 1, and which illustrates in greater detail its mechanism of operation;

FIG. 3 is a front-end view of a writing array for imaging in accordance with the present invention, and in which imaging elements are arranged in a diagonal array;

FIG. 4 is an isometric view of the cylindrical embodiment of an imaging apparatus in accordance with the present invention, and which operates in conjunction with a linear-array writing array;

FIG. 5 is an isometric view of the front of a writing array for imaging in accordance with the present invention, and in which imaging elements are arranged in a linear array;

FIG. 6 is a side view of the writing array depicted in FIG. 5;

FIG. 7 is an isometric view of the flatbed embodiment of an imaging apparatus having a linear lens array;

FIG. 8 is an isometric view of the interior-drum embodiment of an imaging apparatus having a linear lens array;

FIG. 9 is a cutaway view of a remote laser and beam-guiding system;

FIG. 10 is an enlarged, partial cutaway view of a lens element for focusing a laser beam from an optical fiber onto the surface of a printing plate;

FIG. 11 is an enlarged, cutaway view of a lens element having an integral laser;

FIG. 12 is a schematic circuit diagram of a laser-driver circuit suitable for use with the present invention; and

FIGS. 13-16 are enlarged sectional views showing lithographic plates imageable in accordance with the present invention.

#### DETAILED DESCRIPTION OF THE PREFERRED EMBODIMENTS

##### 1. Imaging Apparatus

###### a. Exterior-Drum Recording

Refer first to FIG. 1 of the drawings, which illustrates the exterior drum embodiment of our imaging system. The assembly includes a cylinder 50 around which is wrapped a lithographic plate blank 55. Cylinder 50 includes a void segment 60, within which the outside margins of plate 55 are secured by conventional clamping means (not shown). We note that the size of the void segment can vary greatly depending on the environment in which cylinder 50 is employed.

If desired, cylinder 50 is straightforwardly incorporated into the design of a conventional lithographic press, and serves as the plate cylinder of the press. In a typical press

construction, plate 55 receives ink from an ink train, whose terminal cylinder is in rolling engagement with cylinder 50. The latter cylinder also rotates in contact with a blanket cylinder, which transfers ink to the recording medium. The press may have more than one such printing assembly arranged in a linear array. Alternatively, a plurality of assemblies may be arranged about a large central impression cylinder in rolling engagement with all of the blanket cylinders.

The recording medium is mounted to the surface of the impression cylinder, and passes through the nip between that cylinder and each of the blanket cylinders. Suitable central-impression and in-line press configurations are described in U.S. Pat. No. 5,163,368 (commonly owned with the present application and hereby incorporated by reference) and the '075 patent.

Cylinder 50 is supported in a frame and rotated by a standard electric motor or other conventional means (illustrated schematically in FIG. 2). The angular position of cylinder 50 is monitored by a shaft encoder (see FIG. 4). A writing array 65, mounted for movement on a lead screw 67 and a guide bar 69, traverses plate 55 as it rotates. Axial movement of writing array 65 results from rotation of a stepper motor 72, which turns lead screw 67 and thereby shifts the axial position of writing array 55. Stepper motor 72 is activated during the time writing array 65 is positioned over void 60, after writing array 65 has passed over the entire surface of plate 55. The rotation of stepper motor 72 shifts writing array 65 to the appropriate axial location to begin the next imaging pass.

The axial index distance between successive imaging passes is determined by the number of imaging elements in writing array 65 and their configuration therein, as well as by the desired resolution. As shown in FIG. 2, a series of laser sources  $L_1, L_2, L_3 \dots L_n$ , driven by suitable laser drivers collectively designated by reference numeral 75 (and discussed in greater detail below), each provide output to a fiber-optic cable. The lasers are preferably gallium-arsenide models, although any high-speed lasers that emit in the near infrared region can be utilized advantageously.

The size of an image feature (i.e., a dot, spot or area) and image resolution can be varied in a number of ways. The laser pulse must be of sufficient power and duration to produce useful ablation for imaging; however, there exists an upper limit in power levels and exposure times above which further useful, increased ablation is not achieved. Unlike the lower threshold, this upper limit depends strongly on the type of plate to be imaged.

Variation within the range defined by the minimum and upper parameter values can be used to control and select the size of image features. In addition, so long as power levels and exposure times exceed the minimum, feature size can be changed simply by altering the focusing apparatus (as discussed below). The final resolution or print density obtainable with a given-sized feature can be enhanced by overlapping image features (e.g., by advancing the writing array an axial distance smaller than the diameter of an image feature). Image-feature overlap expands the number of gray scales achievable with a particular feature.

The final plates should be capable of delivering at least 1,000, and preferably at least 50,000 printing impressions. This requires fabrication from durable material, and imposes certain minimum power requirements on the laser sources. For a laser to be capable of imaging the plates described below, its power output should be at least 0.2 megawatt/in<sup>2</sup> and preferably at least 0.6 megawatt/in<sup>2</sup>. Significant ablation

ordinarily does not occur below these power levels, even if the laser beam is applied for an extended time.

Because feature sizes are ordinarily quite small—on the order of 0.5 to 2.0 mils—the necessary power intensities are readily achieved even with lasers having moderate output levels (on the order of about 1 watt); a focusing apparatus, as discussed below, concentrates the entire laser output onto the small feature, resulting in high effective energy densities.

The cables that carry laser output are collected into a bundle 77 and emerge separately into writing array 65. It may prove desirable, in order to conserve power, to maintain the bundle in a configuration that does not require bending above the fiber's critical angle of refraction (thereby maintaining total internal reflection); however, we have not found this necessary for good performance.

Also as shown in FIG. 2, a controller 80 actuates laser drivers 75 when the associated lasers reach appropriate points opposite plate 55, and in addition operates stepper motor 72 and the cylinder drive motor 82. Laser drivers 75 should be capable of operating at high speed to facilitate imaging at commercially practical rates. The drivers preferably include a pulse circuit capable of generating at least 40,000 laser-driving pulses/second, with each pulse being relatively short, i.e., on the order of 10–15  $\mu$ sec (although pulses of both shorter and longer durations have been used with success). A suitable design is described below.

Controller 80 receives data from two sources. The angular position of cylinder 50 with respect to writing array 65 is constantly monitored by a detector 85 (described in greater detail below), which provides signals indicative of that position to controller 80. In addition, an image data source (e.g., a computer) also provides data signals to controller 80. The image data define points on plate 55 where image spots are to be written. Controller 80, therefore, correlates the instantaneous relative positions of writing array 65 and plate 55 (as reported by detector 85) with the image data to actuate the appropriate laser drivers at the appropriate times during scan of plate 55. The control circuitry required to implement this scheme is well-known in the scanner and plotter art; a suitable design is described in U.S. Pat. No. 5,174,205, commonly owned with the present application and hereby incorporated by reference.

The laser output cables terminate in lens assemblies, mounted within writing array 65, that precisely focus the beams onto the surface of plate 55. A suitable lens-assembly design is described below; for purposes of the present discussion, these assemblies are generically indicated by reference numeral 96. The manner in which the lens assemblies are distributed within writing array 65, as well as the design of the writing array, require careful design considerations. One suitable configuration is illustrated in FIG. 3. In this arrangement, lens assemblies 96 are staggered across the face of body 65. The design preferably includes an air manifold 130, connected to a source of pressurized air and containing a series of outlet ports aligned with lens assemblies 96. Introduction of air into the manifold and its discharge through the outlet ports cleans the lenses of debris during operation, and also purges fine-particle aerosols and mists from the region between lens assemblies 96 and plate surface 55.

The staggered lens design facilitates use of a greater number of lens assemblies in a single head than would be possible with a linear arrangement. And since imaging time depends directly on the number of lens elements, a staggered design offers the possibility of faster overall imaging. Another advantage of this configuration stems from the fact

that the diameter of the beam emerging from each lens assembly is ordinarily much smaller than that of the focusing lens itself. Therefore, a linear array requires a relatively significant minimum distance between beams, and that distance may well exceed the desired printing density. This results in the need for a fine stepping pitch. By staggering the lens assemblies, we obtain tighter spacing between the laser beams and, assuming the spacing is equivalent to the desired print density, can therefore index across the entire axial width of the array. Controller 80 either receives image data already arranged into vertical columns, each corresponding to a different lens assembly, or can progressively sample, in a columnar fashion, the contents of a memory buffer containing a complete bitmap representation of the image to be transferred. In either case, controller 80 recognizes the different relative positions of the lens assemblies with respect to plate 55 and actuates the appropriate laser only when its associated lens assembly is positioned over a point to be imaged.

An alternative array design is illustrated in FIG. 4, which also shows the detector 85 mounted to the cylinder 50. Preferred detector designs are described in the '205 patent. In this case the writing array, designated by reference numeral 150, comprises a long linear body fed by fiber-optic cables drawn from bundle 77. The interior of writing array 150, or some portion thereof, contains threads that engage lead screw 67, rotation of which advances writing array 150 along plate 55 as discussed previously. Individual lens assemblies 96 are evenly spaced a distance B from one another. Distance B corresponds to the difference between the axial length of plate 55 and the distance between the first and last lens assembly; it represents the total axial distance traversed by writing array 150 during the course of a complete scan. Each time writing array 150 encounters void 60, stepper motor 72 rotates to advance writing array 150 an axial distance equal to the desired distance between imaging passes (i.e., the print density). This distance is smaller by a factor of n than the distance indexed by the previously described embodiment (writing array 65), where n is the number of lens assemblies included in writing array 65.

Writing array 150 includes an internal air manifold 155 and a series of outlet ports 160 aligned with lens assemblies 96. Once again, these function to remove debris from the lens assemblies and imaging region during operation.

#### b. Flatbed Recording

The imaging apparatus can also take the form of a flatbed recorder, as depicted in FIG. 7. In the illustrated embodiment, the flatbed apparatus includes a stationary support 175, to which the outer margins of plate 55 are mounted by conventional clamps or the like. A writing array 180 receives fiber-optic cables from bundle 77, and includes a series of lens assemblies as described above. These are oriented toward plate 55.

A first stepper motor 182 advances writing array 180 across plate 55 by means of a lead screw 184, but now writing array 180 is stabilized by a bracket 186 instead of a guide bar. Bracket 186 is indexed along the opposite axis of support 175 by a second stepper motor 188 after each traverse of plate 55 by writing array 180 (along lead screw 184). The index distance is equal to the width of the image swath produced by imagewise activation of the lasers during the pass of writing array 180 across plate 55. After bracket 186 has been indexed, stepper motor 182 reverses direction and imaging proceeds back across plate 55 to produce a new image swath just ahead of the previous swath.

It should be noted that relative movement between writing array 180 and plate 55 does not require movement of

writing array 180 in two directions. Instead, if desired, support 175 can be moved along either or both directions. It is also possible to move support 175 and writing array 180 simultaneously in one or both directions. Furthermore, although the illustrated writing array 180 includes a linear arrangement of lens assemblies, a staggered design is also feasible.

#### c. Interior-Arc Recording

Instead of a flatbed, the plate blank can be supported on an arcuate surface as illustrated in FIG. 8. This configuration permits rotative, rather than linear movement of the writing array and/or the plate.

The interior-arc scanning assembly includes an arcuate plate support 200, to which a blank plate 55 is clamped or otherwise mounted. An L-shaped writing array 205 includes a bottom portion, which accepts a support bar 207, and a front portion containing channels to admit the lens assemblies. In the preferred embodiment, writing array 205 and support bar 207 remain fixed with respect to one another, and writing array 205 is advanced axially across plate 55 by linear movement of a rack 210 mounted to the end of support bar 207. Rack 210 is moved by rotation of a stepper motor 212, which is coupled to a gear 214 that engages the teeth of rack 210. After each axial traverse, writing array 205 is indexed circumferentially by rotation of a gear 220 through which support bar 207 passes and to which it is fixedly engaged. Rotation is imparted by a stepper motor 222, which engages the teeth of gear 220 by means of a second gear 224. Stepper motor 222 remains in fixed alignment with rack 210.

After writing array 205 has been indexed circumferentially, stepper motor 212 reverses direction and imaging proceeds back across plate 55 to produce a new image swath just ahead of the previous swath.

#### d. Output Guide and Lens Assembly

Suitable means for guiding laser output to the surface of a plate blank are illustrated in FIGS. 9-11. Refer first to FIG. 9, which shows a remote laser assembly that utilizes a fiber-optic cable to transmit laser pulses to the plate. In this arrangement a laser source 250 receives power via an electrical cable 252. Laser 250 is seated within the rear segment of a housing 255. Mounted within the forepart of housing are two or more focusing lenses 260a, 260b, which focus radiation emanating from laser 250 onto the end face of a fiber-optic cable 265, which is preferably (although not necessarily) secured within housing 255 by a removable retaining cap 267. Cable 265 conducts the output of laser 250 to an output assembly 270, which is illustrated in greater detail in FIG. 10.

With reference to that figure, fiber-optic cable 265 enters the assembly 270 through a retaining cap 274 (which is preferably removable). Retaining cap 274 fits over a generally tubular body 276, which contains a series of threads 278. Mounted within the forepart of body 276 are two or more focusing lenses 280a, 280b. Cable 265 is carried partway through body 276 by a sleeve 280. Body 276 defines a hollow channel between inner lens 280b and the terminus of sleeve 280, so the end face of cable 265 lies a selected distance A from inner lens 280b. The distance A and the focal lengths of lenses 280a, 280b are chosen so at the normal working distance from plate 55, the beam emanating from cable 265 will be precisely focused on the plate surface. This distance can be altered to vary the size of an image feature.

Body 276 can be secured to writing array 65 in any suitable manner. In the illustrated embodiment, a nut 282 engages threads 278 and secures an outer flange 284 of body

276 against the outer face of writing array 65. The flange may, optionally, contain a transparent window 290 to protect the lenses from possible damage.

Alternatively, the lens assembly may be mounted within the writing array on a pivot that permits rotation in the axial direction (i.e., with reference to FIG. 10, through the plane of the paper) to facilitate fine axial positioning adjustment. We have found that if the angle of rotation is kept to 4° or less, the circumferential error produced by the rotation can be corrected electronically by shifting the image data before it is transmitted to controller 80.

Refer now to FIG. 11, which illustrates an alternative design in which the laser source irradiates the plate surface directly, without transmission through fiber-optic cabling. As shown in the figure, laser source 250 is seated within the rear segment of an open housing 300. Mounted within the forepart of housing 300 are two or more focusing lenses 302a, 302b, which focus radiation emanating from laser 250 onto the surface of plate 55. The housing may, optionally, include a transparent window 305 mounted flush with the open end, and a heat sink 307.

It should be understood that while the preceding discussion of imaging configurations and the accompanying figures have assumed the use of optical fibers, in each case the fibers can be eliminated through use of the embodiment shown in FIG. 11.

#### e. Driver Circuitry

A suitable circuit for driving a diode-type (e.g., gallium arsenide) laser is illustrated schematically in FIG. 12. Operation of the circuit is governed by controller 80, which generates a fixed-pulse-width signal (preferably 5 to 20  $\mu$ sec in duration) to a high-speed, high-current MOSFET driver 325. The output terminal of driver 325 is connected to the gate of a MOSFET 327. Because driver 325 is capable of supplying a high output current to quickly charge the MOSFET gate capacitance, the turn-on and turn-off times for MOSFET 327 are very short (preferably within 0.5  $\mu$ sec) in spite of the capacitive load. The source terminal of MOSFET 327 is connected to ground potential.

When MOSFET 327 is placed in a conducting state, current flows through and thereby activates a laser diode 330. A variable current-limiting resistor 332 is interposed between MOSFET 327 and laser diode 330 to allow adjustment of diode output. Such adjustment is useful, for example, to correct for different diode efficiencies and produce identical outputs in all lasers in the system, or to vary laser output as a means of controlling image size.

A capacitor 334 is placed across the terminals of laser diode 330 to prevent damaging current overshoots, e.g., as a result of wire inductance combined with low laser-diode interelectrode capacitance.

#### 2. Lithographic Printing plates

Refer now to FIGS. 13-16, which illustrate various lithographic plate embodiments that can be imaged using the equipment heretofore described. The plate illustrated in FIG. 13 includes a substrate 400, a layer 404 capable of absorbing infrared radiation, and a surface coating layer 408.

Substrate 400 is preferably strong, stable and flexible, and may be a polymer film, or a paper or metal sheet. Polyester films (in the preferred embodiment, the MYLAR film sold by E.I. duPont de Nemours Co., Wilmington, Del., or, alternatively, the MELINEX film sold by ICI Films, Wilmington, Del.) furnish useful examples. A preferred polyester-film thickness is 0.007 inch, but thinner and thicker versions can be used effectively. Aluminum is a preferred metal

substrate. Paper substrates are typically "saturated" with polymers to impart water resistance, dimensional stability and strength.

For additional strength, it is possible to utilize the approach described in U.S. Pat. No. 5,188,032 (commonly owned with the present application and hereby incorporated by reference). As discussed in that application, a metal sheet can be laminated either to the substrate materials described above, or instead can be utilized directly as a substrate and laminated to absorbing layer 404. Suitable metals, laminating procedures and preferred dimensions and operating conditions are all described in the '032 patent and can be straightforwardly applied to the present context without undue experimentation.

The absorbing layer can consist of a polymeric system that intrinsically absorbs in the near-IR region, or a polymeric coating into which near-IR-absorbing components have been dispersed or dissolved.

Exposure of the foregoing construction to the output of one of our lasers weakens surface layer 408 and ablates absorbing layer 404 in the region of exposure. As noted previously, the weakened surface coating (and any debris remaining from destruction of the absorbing second layer) is removed in a post-imaging cleaning step.

Layers 400 and 408 exhibit opposite affinities for ink or an ink-abhesive fluid. In one version of this plate, surface layer 408 is a silicone polymer that repels ink, while substrate 400 is an oleophilic polyester or aluminum material; the result is a dry plate. In a second, wet-plate version, surface layer 408 is a hydrophilic material such as a polyvinyl alcohol (e.g., the Airvol 125 material supplied by Air Products, Allentown, Pa.), while substrate 400 is both oleophilic and hydrophobic.

#### EXAMPLES 1-7

These examples describe preparation of positive-working dry plates that include silicone coating layers and polyester substrates, which are coated with nitrocellulose materials to form the absorbing layers. The nitrocellulose coating layers include thermoset-cure capability and are produced as follows:

| Component                        | Parts |
|----------------------------------|-------|
| Nitrocellulose                   | 14    |
| Cymel 303                        | 2     |
| 2-Butanone (methyl ethyl ketone) | 236   |

The nitrocellulose utilized was the 30% isopropanol wet 5-6 Sec RS Nitrocellulose supplied by Aqualon Co., Wilmington, Del. Cymel 303 is hexamethoxymethylmelamine, supplied by American Cyanamid Corp.

An IR-absorbing compound is added to this base composition and dispersed therein. Use of the following seven compounds in the proportions that follow resulted in production of useful absorbing layers:

| Component        | Example |     |     |     |     |     |     |
|------------------|---------|-----|-----|-----|-----|-----|-----|
|                  | 1       | 2   | 3   | 4   | 5   | 6   | 7   |
| Parts            |         |     |     |     |     |     |     |
| Base Composition | 252     | 252 | 252 | 252 | 252 | 252 | 252 |
| NaCure 2530      | 4       | 4   | 4   | 4   | 4   | 4   | 4   |
| Vulcan XC-72     | 4       | —   | —   | —   | —   | —   | —   |

13  
-continued

| Component             | Example |   |   |   |   |    |    |
|-----------------------|---------|---|---|---|---|----|----|
|                       | 1       | 2 | 3 | 4 | 5 | 6  | 7  |
| Titanium Carbide      | —       | 4 | — | — | — | —  | —  |
| Silicon               | —       | — | 6 | — | — | —  | —  |
| Heliogen Green L 8730 | —       | — | — | 8 | — | —  | —  |
| Nigrosine Base NG-1   | —       | — | — | — | 8 | —  | —  |
| Tungsten Oxide        | —       | — | — | — | — | 20 | —  |
| Manganese Oxide       | —       | — | — | — | — | —  | 30 |

NaCure 2530, supplied by King Industries, Norwalk, Conn., is an amine-blocked p-toluenesulfonic acid solution in an isopropanol/methanol blend. Vulcan XC-72 is a conductive carbon black pigment supplied by the Special Blacks Division of Cabot Corp., Waltham, Mass. The titanium carbide used in Example 2 was the Cerex submicron TiC powder supplied by Baikowski International Corp., Charlotte, N.C. Heliogen Green L 8730 is a green pigment supplied by BASF Corp., Chemicals Division, Holland, Mich. Nigrosine Base NG-1 is supplied as a powder by N H Laboratories, Inc., Harrisburg, Pa.

Following addition of the IR absorber and dispersion thereof in the base composition, the blocked PTSA catalyst was added, and the resulting mixtures applied to the polyester substrate using a wire-wound rod. After drying to remove the volatile solvent(s) and curing (1 min at 300° F. in a lab convection oven performed both functions), the coatings were deposited at 1 g/m<sup>2</sup>.

The nitrocellulose thermoset mechanism performs two functions, namely, anchorage of the coating to the polyester substrate and enhanced solvent resistance (of particular concern in a pressroom environment).

The following silicone coating was applied to each of the anchored IR-absorbing layers produced in accordance with the seven examples described above.

| Component      | Parts |
|----------------|-------|
| PS-445         | 22.56 |
| PC-072         | .70   |
| VM & P Naphtha | 76.70 |
| Syl-Off 7367   | .04   |

(These components are described in greater detail, and their sources indicated, in the '032 patent, cols. 21-23 and also in U.S. Pat. No. 5,212,048, cols. 10 and 11 commonly owned with the present invention and hereby incorporated by reference.)

We applied the mixture using a wire-wound rod, then dried and cured it to produce a uniform coating deposited at 2 g/m<sup>2</sup>. The plates are then ready to be imaged.

## EXAMPLES 8-9

The following examples describe preparation of a plate using an aluminum substrate.

| Component       | Example |    |
|-----------------|---------|----|
|                 | 8       | 9  |
|                 | Parts   |    |
| Ucar Vinyl VMCH | 10      | 10 |
| Vulcan XC-72    | 4       | —  |

14  
-continued

| Component   | Example |     |
|-------------|---------|-----|
|             | 8       | 9   |
| Cymel 303   | —       | 1   |
| NaCure 2530 | —       | 4   |
| 2-Butanone  | 190     | 190 |

Ucar Vinyl VMCH is a carboxy-functional vinyl terpolymer supplied by Union Carbide Chemicals & Plastics Co., Danbury, Conn.

In both examples, we coated a 5-mil aluminum sheet (which had been cleaned and degreased) with one of the above coating mixtures using a wire-wound rod, and then dried the sheets for 1 min at 300° F. in a lab convection oven to produce application weights of 1.0 g/m<sup>2</sup> for Example 8 and 0.5 g/m<sup>2</sup> for Example 9.

For Example 8, we overcoated the dried sheet with the silicone coating described in the previous examples to produce a dry plate.

For Example 9, the coating described above served as a primer (shown as layer 410 in FIG. 14). Over this coating we applied the absorbing layer described in Example 1, and we then coated this absorbing layer with the silicone coating described in the previous examples. The result, once again, is a useful dry plate with the structure illustrated in FIG. 14.

## EXAMPLE 10

Another aluminum plate is prepared by coating an aluminum 7-mil "full hard" 3003 alloy (supplied by All-Foils, Brooklyn Heights, Ohio) substrate with the following formulation (based on an aqueous urethane polymer dispersion) Using a wire-wound rod:

| Component    | Parts |
|--------------|-------|
| NeoRez R-960 | 65    |
| Water        | 28    |
| Ethanol      | 5     |
| Cymel 385    | 2     |

NeoRez R-960, supplied by ICI Resins US, Wilmington, Mass., is an aqueous urethane polymer dispersion. Cymel 385 is a high-methylol-content hexamethoxymethylmelamine, supplied by American Cyanamid Corp.

The applied coating is dried for 1 min at 300° F. to produce an application weight of 1.0 g/m<sup>2</sup>. Over this coating, which serves as a primer, we applied the absorbing layer described in Example 1 and dried it to produce an application weight of 1.0 g/m<sup>2</sup>. We then coated this absorbing layer with the silicone coating described in the previous examples to produce a useful dry plate.

Although it is possible to avoid the use of a priming layer, as was done in Example 8, the use of primers has achieved wide commercial acceptance. Photosensitive dry plates are usually produced by priming an aluminum layer, and then coating the primed layer with a photosensitive layer and then a silicone layer. We expect that priming approaches used in conventional lithographic plates would also serve in the present context.

## EXAMPLES 11-12

In the following examples, we prepared absorbing layers from conductive polymer dispersions known to absorb in the near-IR region. Once again, these layers were formulated to

adhere to a polyester film substrate, and were overcoated with a silicone coating to produce positive-working, dry printing plates.

| Component                   | Example |     | 5  |
|-----------------------------|---------|-----|----|
|                             | 11      | 12  |    |
|                             | Parts   |     |    |
| 5% ICP-117 in Ethyl Acetate | 200     | —   | 10 |
| 5-6 Sec RS Nitrocellulose   | 8       | —   |    |
| Americhem Green #34384-C3   | —       | 100 |    |
| 2-Butanone                  | —       | 100 |    |

The ICP-117 is a proprietary polypyrrole-based conductive polymer supplied by Polaroid Corp. Commercial Chemicals, Assonet, Mass. Americhem Green #34384-C3 is a proprietary polyaniline-based conductive coating supplied by Americhem, Inc., Cuyahoga Falls, Ohio.

The mixtures were each applied to a polyester film using a wire-wound rod and dried to produce a uniform coating deposited at 2 g/m<sup>2</sup>.

#### EXAMPLES 13-14

These examples illustrate use of absorbing layers containing IR-absorbing dyes rather than pigments. Thus, the nigrosine compound present as a solid in Example 5 is utilized here in solubilized form.

| Component                 | Example |     | 25 |
|---------------------------|---------|-----|----|
|                           | 13      | 14  |    |
|                           | Parts   |     |    |
| 5-6 Sec RS Nitrocellulose | 14      | 14  |    |
| Cymel 303                 | 2       | 2   |    |
| 2-Butanone                | 236     | 236 |    |
| Projet 900 NP             | 4       | —   |    |
| Nigrosine Oleate          | —       | 8   | 30 |
| Nacure 2530               | 4       | 4   |    |

Projet 900 NP is a proprietary IR absorber marketed by ICI Colours & Fine Chemicals, Manchester, United Kingdom. Nigrosine oleate refers to a 33% nigrosine solution in oleic acid supplied by N H Laboratories, Inc., Harrisburg, Pa.

The mixtures were each applied to a polyester film using a wire-wound rod and dried to produce a uniform coating deposited at 1 g/m<sup>2</sup>. A silicone layer was applied thereto to produce a working plate.

Substitutions may be made in all of the foregoing Examples 1-14. For example, the melamine-formaldehyde crosslinker (Cymel 303) can be replaced with any of a variety of isocyanate-functional compounds, blocked or otherwise, that impart comparable solvent resistance and adhesion properties; useful substitute compounds include the Desmodur blocked polyisocyanate compounds supplied by Mobay Chemical Corp., Pittsburgh, Pa. Grades of nitrocellulose other than the one used in the foregoing examples can also be advantageously employed, the range of acceptable grades depending primarily on coating method.

#### EXAMPLES 15-16

These examples provide coatings based on polymers other than nitrocellulose, but which adhere to polyester film and can be overcoated with silicone to produce dry plates.

| Component           | Example |     |
|---------------------|---------|-----|
|                     | 15      | 16  |
|                     | Parts   |     |
| Ucar Vinyl VAGH     | 10      | —   |
| Saran F-310         | —       | 10  |
| Vulcan XC-72        | 4       | —   |
| Nigrosine Base NG-1 | —       | 4   |
| 2-Butanone          | 190     | 190 |

Ucar Vinyl VAGH is a hydroxy-functional vinyl terpolymer supplied by Union Carbide Chemicals & Plastics Co., Danbury, Conn. Saran F-310 is a vinylidenedichloride-acrylonitrile copolymer supplied by Dow Chemical Co., Midland, Mich.

The mixtures were each applied to a polyester film using a wire-wound rod and dried to produce a uniform coating deposited at 1 g/m<sup>2</sup>. A silicone layer was applied thereto to produce a working dry plate.

To produce a wet plate, the polyvinylidenedichloride-based I polymer of Example 16 is used as a primer and coated onto the coating of Example 1 as follows:

| Component   | Parts |
|-------------|-------|
| Saran F-310 | 5     |
| 2-Butanone  | 95    |

The primer is prepared by combining the foregoing ingredients and is applied to the coating of Example 1 using a wire-wound rod. The primed coating is dried for 1 min at 300° F. in a lab convection oven for an application weight of 0.1 g/m<sup>2</sup>.

A hydrophilic plate surface coating is then created using the following polyvinyl alcohol solution:

| Component  | Parts |
|------------|-------|
| Airvol 125 | 5     |
| Water      | 95    |

Airvol 125 is a highly hydrolyzed polyvinyl alcohol supplied by Air Products, Allentown, Pa.

This coating solution is applied with a wire-wound rod to the primed, coated substrate, which is dried for 1 min at 300° F. in a lab convection oven. An application weight of 1 g/m<sup>2</sup> yields a wet printing plate capable of approximately 10,000 impressions.

It should be noted that polyvinyl alcohols are typically produced by hydrolysis of polyvinyl acetate polymers. The degree of hydrolysis affects a number of physical properties, including water resistance and durability. Thus, to assure adequate plate durability, the polyvinyl alcohols used in the present invention reflect a high degree of hydrolysis as well as high molecular weight. Effective hydrophilic coatings are sufficiently crosslinked to prevent redissolution as a result of exposure to fountain solution, but also contain fillers to produce surface textures that promote wetting. Selection of an optimal mix of characteristics for a particular application is well within the skill of practitioners in the art.

#### EXAMPLE 17

The polyvinyl-alcohol surface-coating mixture described in the previous example is applied directly to the anchored coating described in Example 13 using a wire-wound rod,

and is then dried for 1 min at 300° F. in a lab convection oven. An application weight of 1 g/m<sup>2</sup> yields a wet printing plate capable of approximately 10,000 impressions.

Various other plates can be fabricated by replacing the Nigrosine Base NG-1 of Example 16 with carbon black (Vulcan XC72) or Heliogen Greeen L 8730.

#### EXAMPLE 18

A layer of indium tin oxide was sputtered onto a polyester film to a thickness sufficient to achieve a resistance of 25–50 ohms/square. A silane primer (glycidoxypropyltrimethoxysilane, supplied by Dow Corning under the trade designation Z-6040) was then applied to this layer and coated with silicone. The result was a nearly transparent, imageable dry plate.

Refer now to FIG. 15, which illustrates a two-layer plate embodiment including a substrate 414 and a surface layer 416. In this case, surface layer 416 absorbs infrared radiation. Our preferred dry-plate variation of this embodiment includes a silicone surface layer 416 that contains a dispersion of IR-absorbing pigment or dye. We have found that many of the surface layers described in U.S. Pat. No. 5,109,771, 5,165,345 and 5,249,525 (all (commonly owned with the present application and hereby incorporated by reference), which contain filler particles that assist the spark-imaging process, can also serve as an IR-absorbing surface layer. In fact, the only filler pigments totally unsuitable as IR absorbers are those whose surface morphologies result in highly reflective surfaces. Thus, white particles such as TiO<sub>2</sub> and ZnO, and off-white compounds such as SnO<sub>2</sub>, owe their light shadings to efficient reflection of incident light, and prove unsuitable for use.

Among the particles suitable as IR absorbers, direct correlation does not exist between performance in the present environment and the degree of usefulness as a spark-discharge plate filler. Indeed, a number of compounds of limited advantage to spark-discharge imaging absorb IR radiation quite well. Semiconductive compounds appear to exhibit, as a class, the best performance characteristics for the present invention. Without being bound to any particular theory or mechanism, we believe that electrons energetically located in and adjacent to conducting bands are readily promoted into and within the band by absorbing IR radiation, a mechanism in agreement with the known tendency of semiconductors to exhibit increased conductivity upon heating due to thermal promotion of electrons into conducting bands.

Currently, it appears that metal borides, carbides, nitrides, carbonitrides, bronze-structured oxides, and oxides structurally related to the bronze family but lacking the A component (e.g., WO<sub>2.9</sub>) perform best.

IR absorption can be further improved by adding an IR-reflective surface below the IR-absorbing layer. This approach provides maximum improvement to embodiments in which the absorbing layer is itself ablated, i.e., the plates illustrated in FIGS. 13 and 15. FIG. 16 illustrates introduction of a reflective aluminum layer 418 between layers 416 and 414. To produce a dry plate having this reflective layer, a thin layer of aluminum from 200 to 700 angstroms thick is deposited directly onto substrate 414; suitable means of deposition, as well as alternative materials, are described in connection with layer 178 of FIG. 4F in the '075 patent mentioned earlier. The silicone coating is then applied to layer 418 in the same manner described above. Exposure to the laser beam results in ablation of layer 416. In a similar

fashion, a thin metal layer can be interposed between layers 404 and 400 of the plate illustrated in FIG. 13.

Silicone coating formulations particularly suitable for deposition onto an aluminum layer are described in the '032 and '048 patents. In particular, commercially prepared pigment/gum dispersions can be advantageously utilized in conjunction with a second, lower-molecular-weight second component.

In the following coating examples, the pigment/gum mixtures, all based on carbon-black pigment, are obtained from Wacker Silicones Corp., Adrian, Mich. In separate procedures, coatings are prepared using PS-445 and dispersions marketed under the designations C-968, C-1022 and C-1190 following the procedures outlined in the '032 and '048 patents. The following formulations are utilized to prepare stock coatings:

| Order of Addition | Component              | Weight Percent |
|-------------------|------------------------|----------------|
| 1                 | VM & P Naphtha         | 74.8           |
| 2                 | PS-445                 | 15.0           |
| 3                 | Pigment/Gum Dispersion | 10.0           |
| 4                 | Methyl Pentynol        | 0.1            |
| 5                 | PC-072                 | 0.1            |

Coating batches are then prepared as described in the '032 and '048 patents applications using the following proportions:

| Component       | Parts |
|-----------------|-------|
| Stock Coating   | 100   |
| VM & P Naphtha  | 100   |
| PS-120 (Part B) | 0.6   |

The coatings are straightforwardly applied to the aluminum layers, and contain useful IR-absorbing material.

It will therefore be seen that we have developed a highly versatile imaging system and a variety of plates for use therewith. The terms and expressions employed herein are used as terms of description and not of limitation, and there is no intention, in the use of such terms and expressions, of excluding any equivalents of the features shown and described or portions thereof, but it is recognized that various modifications are possible within the scope of the invention claimed.

What is claimed is:

1. Printing apparatus comprising:
  - a. a printing member having a printing surface and including a solid oleophobic layer and a solid oleophilic layer underlying the oleophobic layer, one of said layers being characterized by ablative absorption of imaging radiation;
  - b. means for supporting the printing member;
  - c. at least one laser source that produces an imaging output;
  - d. means for guiding the output of the at least one laser source to focus on the printing surface;
  - e. means for causing relative movement between the guiding means and support means to effect a scan of the printing surface by the laser output;
  - f. means for selectively actuating, in a pattern representing an image, the laser source so as to ablate the absorptive layer, thereby removing or facilitating removal of the oleophobic layer; and

- g. means for mechanically removing, without a cleaning solvent, the oleophobic layer where the absorptive layer has been ablated.
2. The apparatus of claim 1 wherein the selectable actuation means includes a pulse circuit that operates at speeds of at least 40,000 pulses/second. 5
3. The apparatus of claim 1 wherein each laser source outputs a power level of at least 0.2 megawatt/in<sup>2</sup>.
4. The apparatus of claim 1 wherein each laser source emits primarily in the near-IR region. 10
5. The apparatus of claim 1 wherein each laser source is an infrared semiconductor laser.
6. Printing apparatus comprising:
- a. at least one print station including:
  - i. a plate cylinder;
  - ii. a printing plate having a printing surface and including a solid oleophobic layer and a solid oleophilic layer underlying the oleophobic layer, one of said layers being characterized by ablative absorption of imaging radiation; 15
  - iii. means for mounting the plate to the plate cylinder;
  - iv. at least one laser source that produces an imaging output;
  - v. means for guiding the output of the at least one laser source to focus on the printing surface; 20
  - vi. means for causing relative movement between the guiding means and plate to effect a scan of the printing surface by the laser output;
  - vii. means for selectively actuating, in a pattern representing an image, the laser source so as to ablate the absorptive layer, thereby removing or facilitating removal of the oleophobic plate layer and directly producing on the plate an array of image features; 25
  - viii. means for mechanically removing, without a cleaning solvent, the oleophobic layer where the absorptive layer has been ablated; and 30
- b. means for transferring a recording medium to the print station.
7. The apparatus of claim 6 wherein the apparatus comprises a plurality of print stations arranged in an in-line configuration. 40
8. The apparatus of claim 6 wherein the apparatus comprises a plurality of print stations arranged in a central-impression configuration. 45
9. Printing apparatus comprising:
- a. a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation; 50
  - b. at least one laser source that produces an imaging output;
  - c. means for guiding the output of the at least one laser source to focus on the printing surface; 60
  - d. means for causing relative movement between the guiding means and the member to effect a scan of the printing surface by the laser output;
  - e. means for selectively actuating, in a pattern representing an image, the laser source so as to ablate the absorptive layer, thereby removing or facilitating removal of the second layer; and 65

- f. means for mechanically removing, without a cleaning solvent, the first layer where the second layer has been ablated.
10. The apparatus of claim 9 wherein the substrate is oleophilic and the first layer is oleophobic.
11. The apparatus of claim 9 wherein the selectable actuation means includes a pulse circuit that operates at speeds of at least 40,000 pulses/second.
12. The apparatus of claim 9 wherein each laser source outputs a power level of at least 0.2 megawatt/in<sup>2</sup>. 10
13. The apparatus of claim 9 wherein each laser source emits primarily in the near-IR region.
14. The apparatus of claim 9 wherein each laser source is an infrared semiconductor laser.
15. Printing apparatus comprising:
- a. at least one print station including:
  - i. a plate cylinder;
  - ii. a printing plate having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation; 15
  - iii. means for mounting the plate to the plate cylinder;
  - iv. at least one laser source that produces an imaging output;
  - v. means for guiding the output of the at least one laser source to focus on the printing surface; 20
  - vi. means for causing relative movement between the guiding means and the plate to effect a scan of the printing surface by the laser output;
  - vii. means for selectively actuating, in a pattern representing an image, the laser source so as to ablate the absorptive layer, thereby removing or facilitating removal of the second layer; and 25
  - viii. means for mechanically removing, without a cleaning solvent, the first layer where the second layer has been ablated; and 30
- b. means for transferring a recording medium to the print station.
16. The apparatus of claim 15 wherein the substrate is oleophilic and the first layer is oleophobic.
17. The apparatus of claim 15 wherein the apparatus comprises a plurality of print stations arranged in an in-line configuration. 45
18. The apparatus of claim 15 wherein the apparatus comprises a plurality of print stations arranged in a central-impression configuration. 50
19. Printing apparatus comprising:
- a. a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation; 55
  - b. at least one laser source that produces an imaging output;
  - c. means for guiding the output of the at least one laser source to focus on the printing surface; 60
  - d. means for causing relative movement between the guiding means and the member to effect a scan of the printing surface by the laser output;

- e. means for selectively actuating, in a pattern representing an image, the laser source so as to ablate the absorptive layer, thereby removing or facilitating removal of the second layer; and
- f. means for mechanically removing the first layer where the second layer has been ablated, wherein the substrate is hydrophobic and the first layer is hydrophilic.

20. The apparatus of claim 19 wherein the substrate is also oleophilic.

21. Printing apparatus comprising:

- a. at least one print station including:
  - i. a plate cylinder;
  - ii. a printing plate having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation;
  - iii. means for mounting the plate to the plate cylinder;
  - iv. at least one laser source that produces an imaging output;
  - v. means for guiding the output of the at least one laser source to focus on the printing surface;
  - vi. means for causing relative movement between the guiding means and the plate to effect a scan of the printing surface by the laser output;
  - vii. means for selectively actuating, in a pattern representing an image, the laser source so as to ablate the absorptive layer, thereby removing or facilitating removal of the second layer; and
  - viii. means for mechanically removing the first layer where the second layer has been ablated; and
- b. means for transferring a recording medium to the print station;

wherein the substrate is hydrophobic and the first layer is hydrophilic.

22. The apparatus of claim 21 wherein the substrate is also oleophilic.

23. A method of imaging a lithographic printing member, the method comprising the steps of:

- a. providing a printing member having a printing surface and including a solid oleophobic layer and a solid oleophilic layer underlying the oleophobic layer, one of said layers being characterized by ablative absorption of imaging radiation;
- b. spacing at least one laser source that produces an imaging output opposite the printing surface;
- c. guiding the output of the at least one laser source to focus on the printing surface;
- d. causing relative movement between the laser output and the printing member to effect a scan of the printing surface by the laser output; and
- e. selectively exposing, in a pattern representing an image, the printing surface to the laser output during the course of the scan so as to ablate the absorptive layer, thereby removing or facilitating removal of the oleophobic layer; and
- f. mechanically removing, without a cleaning solvent, remaining portions of the oleophobic layer where the absorptive layer has been ablated.

24. The method of claim 23 wherein the selective-exposure step occurs at a rate of at least 40,000 pulses/second.

25. The method of claim 23 wherein each laser source emits primarily in the near-infrared region.

26. The method of claim 23 wherein each laser source is a semiconductor laser.

27. A method of printing with a printing press that includes a plate cylinder, the method comprising the steps of:

- a. providing a printing plate having a printing surface and including a solid oleophobic layer and a solid oleophilic layer underlying the oleophobic layer, one of said layers being characterized by ablative absorption of imaging radiation;
- b. mounting the plate to the plate cylinder;
- c. spacing at least one laser source that produces an imaging output opposite the printing surface of the plate;
- d. guiding the output of the at least one laser source to focus on the printing surface;
- e. causing relative movement between the laser output and the printing plate to effect a scan of the printing surface by the laser output;
- f. selectively exposing, in a pattern representing an image, the printing surface to the laser output during the course of the scan so as to ablate the absorptive layer, thereby removing or facilitating removal of the oleophobic plate layer;
- g. mechanically removing, without a cleaning solvent, remaining portions of the oleophobic layer where the absorptive layer has been ablated;
- h. applying ink to the plate; and
- i. transferring the ink to a recording medium.

28. The method of claim 27 wherein the selective-exposure step occurs at a rate of at least 40,000 pulses/second.

29. The method of claim 27 wherein each laser source emits primarily in the near-infrared region.

30. The method of claim 27 wherein each laser source is a semiconductor laser.

31. A method of imaging a lithographic printing member, the method comprising the steps of:

- a. providing a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation;
- b. spacing at least one laser source that produces an imaging output opposite the printing surface of the printing member;
- c. guiding the output of the at least one laser source to focus on the printing surface;
- d. causing relative movement between the laser output and the printing member to effect a scan of the printing surface; and
- e. selectively exposing, in a pattern representing an image, the printing surface to the laser output during the course of the scan so as to selectively remove or facilitate removal of, in a pattern representing an image, the first and second layers, thereby ablating the second layer; and
- f. mechanically removing, without a cleaning solvent, remaining portions of the first layer where the second layer has been ablated.

32. The method of claim 31 wherein the substrate is oleophilic and the first layer is oleophobic.

33. The method of claim 31 wherein the selective-exposure step occurs at a rate of at least 40,000 pulses/second.

34. The method of claim 31 wherein each laser source emits primarily in the near-infrared region.

35. The method of claim 31 wherein each laser source is a semiconductor laser.

36. A method of printing with a printing press that includes means for supporting a lithographic printing member, the method comprising the steps of:

- a. providing a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation;
- b. mounting the printing member to the support means;
- c. spacing at least one laser source that produces an imaging output opposite the printing surface of the printing member;
- d. guiding the output of the at least one laser source to focus on the printing surface;
- e. causing relative movement between the laser output and support means to effect a scan of the printing surface;
- f. selectively exposing, in a pattern representing an image, the printing surface to the laser output during the course of the scan so as to selectively remove or facilitate removal of the first and second layers, thereby ablating the second layer;
- g. mechanically removing, without a cleaning solvent, remaining portions of the first layer where the second layer has been ablated;
- h. applying ink to the member; and
- i. transferring the ink to a recording medium.

37. The method of claim 36 wherein the substrate is oleophilic and the first layer is oleophobic.

38. The method of claim 36 wherein the selective-exposure step occurs at a rate of at least 40,000 pulses/second.

39. The method of claim 36 wherein each laser source emits primarily in the near-infrared region.

40. The method of claim 36 wherein each laser source is a semiconductor laser.

41. A method of imaging a lithographic printing member, the method comprising the steps of:

- a. providing a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation;

b. spacing at least one laser source that produces an imaging output opposite the printing surface of the printing member;

c. guiding the output of the at least one laser source to focus on the printing surface;

d. causing relative movement between the laser output and the printing member to effect a scan of the printing surface; and

e. selectively exposing, in a pattern representing an image, the printing surface to the laser output during the course of the scan so as to selectively remove or facilitate removal of, in a pattern representing an image, the first and second layers, thereby ablating the second layer; and

f. mechanically removing remaining portions of the first layer where the second layer has been ablated, wherein the substrate is hydrophobic and the first layer is hydrophilic.

42. The method of claim 41 wherein the substrate is also oleophilic.

43. A method of printing with a printing press that includes means for supporting a lithographic printing member, the method comprising the steps of:

- a. providing a printing member having a printing surface and including a first solid layer, a second solid layer underlying the first layer, and a solid substrate underlying the second layer, the first layer and substrate having different affinities for at least one printing liquid selected from the group consisting of ink and an adhesive fluid for ink, the second layer, but not the first layer, being formed of a material being subject to ablative absorption of imaging radiation;

- b. mounting the printing member to the support means;
- c. spacing at least one laser source that produces an imaging output opposite the printing surface of the printing member;

- d. guiding the output of the at least one laser source to focus on the printing surface;

- e. causing relative movement between the laser output and support means to effect a scan of the printing surface;

- f. selectively exposing, in a pattern representing an image, the printing surface to the laser output during the course of the scan so as to selectively remove or facilitate removal of the first and second layers, thereby ablating the second layer;

- g. mechanically removing, without a cleaning solvent, remaining portions of the first layer where the second layer has been ablated;

- h. applying ink to the member; and

- i. transferring the ink to a recording medium, wherein the substrate is hydrophobic and the first layer is hydrophilic.

44. The method of claim 43 wherein the substrate is also oleophilic.

UNITED STATES PATENT AND TRADEMARK OFFICE  
CERTIFICATE OF CORRECTION

PATENT NO. : 5,540,150

DATED : July 30, 1996

INVENTOR(S) : Thomas E. Lewis et al.

It is certified that error appears in the above-identified patent and that said Letters Patent is hereby corrected as shown below:

In col. 13, line 42, change ".70" to --.04--; and  
at line 44, change ".04" to --.70--

Signed and Sealed this

Ninth Day of September, 1997

Attest:



BRUCE LEHMAN

Attesting Officer

Commissioner of Patents and Trademarks